

1

2,899,306

## ANTIFOGGANTS FOR REVERSAL COLOR DEVELOPMENT

Catherine Marilyn Spath, Rochester, N.Y., assignor to Eastman Kodak Company, Rochester, N.Y., a corporation of New Jersey

No Drawing. Application January 24, 1957  
Serial No. 635,944

10 Claims. (Cl. 96—56)

This invention relates to color photography, and more particularly, to a method of processing multi-layer color films or papers in such a manner as to reduce color fog and give maximum color density. 15

In multi-layer photographic elements used for color photography, there are usually three selectively sensitive emulsion layers coated on one side of a single support. The uppermost layer is generally blue-sensitive, the next layer is generally green-sensitive, while the emulsion layer adjacent the support is generally red-sensitive. Between the blue-sensitive and green-sensitive layers is a filter 20 layer for absorbing blue radiation which may be transmitted through the blue-sensitive layer. The multi-layer coating can also have other interlayers for specialized purposes. Such multi-layer materials have been previously described in the prior art, such as Mannes et al. U.S. Patent 2,252,718, issued August 19, 1941.

Color materials of the type employed in the instant invention are those intended primarily for reversal processes, wherein the exposed material is given a conventional black-and-white development, followed by a reversal exposure, or exposures, and color development. 35

The color materials used in my invention comprise emulsions which can contain color-forming materials or couplers, or these color couplers can be used instead in the color developers.

It is, therefore, an object of my invention to provide improved developers for reversal color photography. Another object is to provide a method of inhibiting color fog and increasing the maximum color density. Other objects will become apparent from a consideration of the following examples and description. 45

During the black-and-white development of multi-layer color materials, fog centers are introduced into the unexposed regions, and upon reversal exposure and subsequent color development, these unexposed areas have deposited therein coupled color-forming materials, resulting in severe loss of color quality. For example, in processing color materials of the Kodachrome type, color developer containing a cyan coupler results not only in development of the red-sensitive layer, but also in development of cyan fog in the blue- and green-sensitive layers. This fog is particularly severe in emulsions which contain conventional chemical sensitizers, such as gold sensitizers, sulfur sensitizers, or polyethyleneglycol type chemical sensitizers.

I have now found that such undesirable fog can be eliminated or materially reduced by adding an organic compound containing a formamidinothiomethyl substituent to one or more of the color developers. These formamidinothiomethyl compounds decrease color fog in the unexposed areas with no substantial loss of color density in the exposed areas. These compounds can be conveniently added to the color developer, which may or may not contain a color coupler or color-forming compound, depending upon the particular color material being 70

2

processed. It is to be understood that my invention comprises the use of color materials which may contain the color couplers or color-forming compounds either in the emulsions or in the color developing solutions. Particular benefits have been obtained with color materials wherein the color couplers or color-forming materials are present in the color developing solutions.

It is known that a colored image can be formed by adding to certain color developing solutions, or by incorporating in the silver halide emulsion, a compound which couples during development with the oxidation product of the developing agent, thus forming a colored compound which is deposited adjacent to the silver grains of the silver image during such development. Such compound which is employed in conjunction with the developing agent for the silver and which couples with the oxidation product of the developing agent during development is referred to as a color-forming compound or coupler. Such compounds usually belong to one of three widely known types, i.e., pyrazolone couplers, phenol couplers, or open-chain ketomethylene couplers. These couplers produce, respectively, magenta, cyan and yellow images.

The formamidinothiomethyl compounds useful in practicing my invention include compounds represented by the following general formula:



wherein R represents a hydrogen atom, an alkyl group (e.g., methyl, ethyl, propyl, etc., especially a lower alkyl group), or an aryl group (e.g., phenyl, tolyl, etc., especially a monocyclic aryl group of the benzene series containing from 6 to 7 carbon atoms), R<sub>1</sub> represents an amino group (e.g., amino, monoalkylamino, such as methylamino, ethylamino, butylamino, etc., dialkylamino, such as dimethylamino, diethylamino, etc., monoarylamino, such as phenylamino, tolylaminio, etc., diarylamino, such as diphenylamino, ditolylamino, etc., heterocyclic amino, such as 2-thiazylamino, triazylamino, etc.), and R<sub>2</sub> represents a carbalkoxyl group (e.g., carbomethoxy, carbethoxyl, carbobutoxyl, etc., especially a carbalkoxyl group containing from 2 to 5 carbon atoms), an alkyl group (e.g., ethyl, n-propyl, n-butyl,  $\beta$ -sulfoethyl, etc., especially an alkyl group containing from 1 to 4 carbon atoms), a heterocyclic group (e.g., tetrazaindenyl, pyridyl, etc.), or an amido group (e.g., amido, 40

45



50 thiazylamido



55 phenylamido



etc., i.e., an aminocarbonyl group).

The formamidinothiomethyl compounds which can advantageously be employed in my invention include the following:

(a)



2-formamidinothiomethyl-4-hydroxy-6-methyl-1,3,3a,7-tetrazaindene



The above formamidinothiomethyl compounds can be prepared according to methods previously described in the art. See, for example, Knott et al. U.S. Patent 2,461,987, issued February 15, 1949, and Tinker et al. U.S. application Serial No. 515,785, filed June 15, 1955 (now U.S. Patent 2,835,581, issued May 20, 1958). Further examples describing the preparation of these compounds are given below.

The formamidinothiomethyl compounds employed in the color developers of my invention can be utilized in various concentrations depending upon the particular emulsions employed, the concentration of silver halides in the emulsions, and the concentration of the developing agents in the developers. In general, not less than about 10 mg. per liter of developer of formamidinothiomethyl compound should be employed. The most advantageous concentration can be determined by developing a series of test strips of silver halide emulsions wherein the concentration of formamidinothiomethyl compound is varied, as well as the concentration of the developing agent. The usual addenda can be employed in the developers, such as strongly alkaline agents, sodium carbonate, potassium carbonate, sodium hydroxide, etc., restraining agents, such as potassium bromide, stain preventives, such as alkali metal sulfites, etc.

My invention is primarily directed to the development of the ordinarily employed gelatino-silver-halide developing-out emulsions, e.g., gelatino-silver-chloride, -chlorobromide, -chloroiodide, -chlorobromiodide, -bromide and -bromiodide developing-out emulsions. While the results in the following examples were obtained using gelatino-silver-bromiodide emulsions, excellent results can also be obtained using other silver halide emulsions. These emulsions can be coated in the usual manner on any suitable support, e.g., glass, cellulose nitrate film, cellulose acetate film, polyvinyl acetal resin film, paper or metal.

Photographic silver halide emulsions useful in my invention can also contain such addenda as chemical sen-

sitzers, e.g., sulfur sensitizers (e.g., allyl thiocarbamide, thiourea, allyl isothiocyanate, cystine, etc.), various gold compounds (e.g., potassium chloroaurate, auric trichloride, etc.) (see U.S. Patents 2,540,085; 2,597,856 and 2,597,915), various azaindene compounds (such as those disclosed in U.S. Patent 2,716,062), condensation products of alkylene oxides, such as those shown in U.S. Patent 2,400,532, as well as the additives mentioned in Jones et al. U.S. application Serial No. 575,160, filed March 30, 1956.

As mentioned above, the advantages of my invention are particularly outstanding in reversal color photographic processes. Couplers or color-forming compounds which are soluble in the strongly alkaline developing solutions are well known to those skilled in the art. Typical couplers include the following:

#### COUPLERS FOR USE IN COLOR DEVELOPERS

##### Cyan couplers:

- 20 1. 5-benzenesulfonamino-1-naphthol  
 2. 2,4-dichloro-5-benzenesulfamino-1-naphthol  
 3. 2,4-dichloro-5-(p-toluenesulfamino)-1-naphthol  
 4. 5-(1,2,3,4-tetrahydronaphthalene-6-sulfonamino)-1-naphthol  
 25 5. 2,4-dichloro-5-(4'-bromodiphenyl-4-sulfonamino)-1-naphthol  
 6. o-( $\beta$ -Naphthalenesulfonamino)-phenol  
 7. 5-(m-nitrobenezenesulfonamino)-1-naphthol  
 8. 5-(quinoline-5-sulfonamino)-1-naphthol  
 (U.S. 2,362,598)  
 30 9. 2-acetylarnino-5-methylphenol  
 10. 2-benzoylarnino-3,5-dimethylphenol  
 11. 2- $\alpha$ -(p-tert. amylophenoxy)-n-butyrylarnino-5-methylphenol  
 12. 2- $\alpha$ -(p-tert. amylophenoxy)-n-butyrylarnino-4-chloro-5-methylphenol  
 13. 2-(p-tert. amylophenoxy-p-benzoyl)arnino-4-chloro-5-methylphenol  
 14. 2-(4'-tert. amylo-3'-phenoxybenzoylarnino)-3,5-dimethyl-1-phenol  
 15. 2-phenylacetylarnino-4-chloro-5-methylphenol  
 16. 2-benzoylarnino-4-chloro-5-methylphenol  
 17. 2-anilinoacetylarnino-4-chloro-5-methylphenol  
 18. 2-{4'-[ $\alpha$ -(4'-tert. amylophenoxy)-n-butyrylarnino]-benzoylarnino}-4-chloro-5-methylphenol  
 19. 2-{4'-[3'-(4'-tert. amylophenoxy)-benzoylarnino]-4-chloro-5-methylphenol  
 20. 2-p-nitrobenzoylarnino-4-chloro-5-methylphenol  
 21. 2-m-aminobenzoyl-4-chloro-5-methylphenol  
 22. 2-acetarnino-4-chloro-5-methylphenol  
 23. 2-(4'-sec. amylobenzarnino)-4-chloro-5-methylphenol  
 24. 2-(4'-n-amyloxybenzarnino)-4-chloro-5-methylphenol

##### Magenta couplers:

- 25 1-phenyl-3-acetylarnino-5-pyrazolone  
 26. 1-phenyl-3-propionylarnino-5-pyrazolone  
 27. 1-phenyl-3-dichloroacetylarnino-5-pyrazolone  
 28. 1-phenyl-3-benzoylarnino-5-pyrazolone  
 29. 1-phenyl-3-(m-aminobenzoyl)arnino-5-pyrazolone hydrochloride  
 30. 1-phenyl-3-(diamylbenzoyl)arnino-5-pyrazolone  
 31. 1-phenyl-3-phenylcarbamylarnino-5-pyrazolone  
 32. 1-phenyl-3-phenoxyacetylarnino-5-pyrazolone  
 33. 1-phenyl-3-p-aminobenzoylarnino-5-pyrazolone  
 34. 1-phenyl-3-(o-carboxybenzoyl)arnino-5-pyrazolone  
 35. 1-phenyl-3-palmitylarnino-5-pyrazolone  
 36. 1-phenyl-3-(p-sec. amylobenzene-sulfonylarnino)-5-pyrazolone  
 37. 1-phenyl-3-[p-(p-sec. amylobenzoyl)arnino-benzoylarnino]-5-pyrazolone

38. 1-m-tolyl-3-[m - ( $\beta$ -phenylpropionyl)aminobenzoylaminol]-5-pyrazolone  
 39. 1 - m - tolyl - 3-(2,4-di-tert. butyl-m-tolylloxy-acetylamino)-5-pyrazolone  
 40. 1 - [p-(p'-tert. butylphenoxy)phenyl]-3-[p-(benzoylaminol)-benzoylaminol]-5-pyrazolone 5  
 41. 1-(p-tert. butylphenoxyphenyl) - 3 - (p-m-amyloxybenzoylaminol)-5-pyrazolone  
 42. 1-[p-(p'-tert. butylphenoxy)phenyl] - 3 - (3,5-dimethoxybenzoyl)amino-5-pyrazolone 10  
 43. 1-[p-(p'-tert. butylphenoxy)phenyl]-3 - [m-(p-toluene-sulfonylaminol)benzoylaminol]-5 - pyrazolone  
 44. 1 - [p-(3,5 - dimethylphenoxy)phenyl]-3-(4-n-amyloxy-3-methylbenzoylaminol)-5-pyrazolone 15  
 45. 3-(p - nitrophenoxyacetamino) - 1-(2',4',6'-trichlorophenyl)-5-pyrazolone

## Yellow couplers:

46. p-( $\omega$ -Benzoylacetamino)benzenesulfonamide  
 47. p - ( $\omega$  - Benzoylacetamino)benzenesulfon - N - 20 methylamide  
 48. p-( $\omega$ -Benzoylacetamino)benzenesulfonanilide  
 49. 4-benzenesulfonamino- $\omega$ -benzoylacetanilide  
 50. 4 - (p-toluenesulfonamino)- $\omega$ -benzoylacetanilide 25  
 51. 4 - (p-laurylbenzenesulfonamino)- $\omega$ -benzoylacetanilide  
 52. 1,4-di - [p - (benzoylacetamino)benzenesulfonamino]benzene  
 53. N,N' - di - (p-benzoylacetaminophenyl)benzene-1,3-disulfonamide  
 54. N - (p - benzoylacetaminophenyl)-4-[p-(benzoylacetamino) - benzenesulfonamido]benzenesulfonamide  
 55. N<sup>4</sup>-benzoylacetyl - N'-(2-benzothiazolyl)sulfanilamide  
 56. p - Acetoacetaminobenzenesulfon- $\beta$ -naphthalide  
 57. p - Furoylacetaminobenzenesulfon-N-cyclohexylamide  
 58. p - (4 - ethoxybenzoylacetamino)benzenesulfonamide  
 59. Terephthaloyl - bis[(p-N-amylsulfonamido)acetanilide]  
 60. p - (Quinoline - 8 - sulfonamino)- $\omega$ -benzoylacetanilide  
 61. p - Acetoacetamino-o-methylbenzenesulfon - N - 45 anilide  
 62. N,N' - di - (p - benzoylacetaminophenol)naphthalene-1,5-disulfonamide  
 63. p-(Benzenesulfonamino)benzoylacetone  
 64. N-benzoylaceto-o-anisidine 50

Typical couplers that are primarily useful in the photographic silver halide emulsion layers of my invention comprise the following:

## Coupler:

65. 1 - hydroxy-2-[ $\delta$ -(2',4'-di-tert.amylphenoxy) - n-butyl]-naphthamide (U.S. Patent 2,474,293)  
 66. 1 - hydroxy - 4-phenylazo-4'-(p-tert.-butylphenoxy)-2-naphthaniide (U.S. Patent 2,521,908)  
 67. 2 - (2,4 - di-tert.-amylphenoxyacetamino)-4,6-di-chloro-5-methylphenol (U.S. Patent 2,725,291)  
 68. 2 - ( $\alpha$  - di-tert.amylphenoxy-n-butylaminol)-4,6-dichloro-t-methylphenol  
 69. 6-{ $\alpha$  - {4 - [ $\alpha$ -(2,4 - di-tert.amylphenoxy)butyramido]phenoxy}acetamido} - 2,4 - dichloro - 3-methylphenol  
 70. 2 - [3'-(2'',4'' - diamylphenoxy) - acetamido]benzamido-4-chloro-5-methylphenol  
 71. 1-(2',4',6' - trichlorophenyl) - 3 - [3''-(2'',4'' - di-tert.-amylphenoxyacetamido) - benzamido] - 5-pyrazolone (U.S. Patent 2,600,788) 70  
 72. 1-(2',4',6' - trichlorophenyl)-3-[3''-(2'',4'' - di-tert.-amylphenoxyacetamido)-benzamido] - 4-(p-methoxyphenyl-azo)-5-pyrazolone

73. N-(4 - benzoylacetaminobenzenesulfonyl) - N-( $\gamma$ -phenylpropyl)-p-toluidine (U.S. Patent 2,298,443)  
 74.  $\alpha$ -o-Methoxybenzoyl- $\alpha$ -chloro - 4-[ $\alpha$ -(2,4-di-tert.-amylphenoxy) - n - butyramido]-acetanilide (McCloskey U.S. Patent 2,728,658)  
 75.  $\alpha$ -{3-[ $\alpha$  - (2,4-di-tert.amylphenoxy)acetamido]-benzoyl}-2-methoxyacetanilide  
 76. 3 - benzoylacetamido - 4 - methoxy-2',4'-di-tert.-amylphenoxyacetanilide  
 77. 4 - benzoylacetamido - 3-methoxy-2',4'-di-tert.-amylphenoxyacetanilide

Other couplers suitable for use in the emulsions of my invention comprise those disclosed in Spence and Carroll U.S. Patent 2,640,776, issued June 2, 1953; Weissberger et al. U.S. Patent 2,407,210, issued September 3, 1946; and Weissberger et al. U.S. Patent 2,474,293, issued June 28, 1949.

The color-forming developers useful in my invention have been previously described in the prior art, and my invention is not to be restricted to the use of any particular color-forming developer. The color-forming developers previously mentioned which I have found to be especially useful in my invention comprise aromatic primary amines containing an amino (substituted or not) or hydroxyl substituent. Phenylenediamines and substituted derivatives thereof containing a primary amino group have been found to provide excellent results when employed in combination with the formamidinothiomethyl compounds of my invention. Typical of such color-forming developers are the sulfonamido substituted p-phenylenediamines disclosed in Weissberger U.S. Patent 2,548,574, issued April 10, 1951, the substituted p-phenylenediamines disclosed in Weissberger et al. U.S. Patent 2,566,271, issued August 28, 1951. Other phenylenediamine color-forming developers can be employed to like advantage in the process of my invention.

The first developer employed in the process of my invention is generally a rapid developer of the MQ type, i.e., a combination of hydroquinone and Elon (p-N-methylaminophenyl) developer.

The photographic silver halide emulsions useful in the process of my invention can be prepared according to known methods, such as those described in Hewitson and McClintock U.S. Patent 2,618,556, issued November 18, 1952. Of course, emulsions prepared by other methods can be used to equal advantage in my invention.

These emulsions can be chemically sensitized or not, as mentioned above. Additional chemical sensitizers useful in my invention comprise those disclosed in the co-pending application Serial No. 550,495, filed December 1, 1955 (now U.S. Patent 2,886,437, issued May 12, 1958), in the name of D. E. Piper.

The following examples will serve to illustrate more fully the manner of practicing my invention.

## Example 1

A portion of a gelatino-silver-bromide emulsion which had been sensitized with a sulfur compound and a gold compound as mentioned above was coated on a cellulose acetate support. The coating was then cut into several strips, identified coating series A below. The oleyl ether of a polyethyleneglycol having a molecular weight greater than 300 was added to a second portion of the same emulsion at a concentration of 5 gms. of the oleyl ether per mole of silver halide, and the emulsion coated onto a cellulose acetate support. The dried coating was then cut into several strips, identified coating series B below. One strip of each coating was exposed for  $\frac{1}{25}$  second to a 500-watt, 3000° K. light source on an Eastman Type Ib sensitometer. The exposed coatings

were then developed for 3 minutes in a developer having the following composition:

|                                  |     |      |
|----------------------------------|-----|------|
| Sodium hexametaphosphate         | g.  | 0.5  |
| Sodium sulfite (anhydrous)       | g.  | 40.0 |
| N-methyl-p-aminophenolsulfate    | g.  | 5.0  |
| Hydroquinone                     | g.  | 2.0  |
| Sodium carbonate (monohydrate)   | g.  | 25.0 |
| Potassium bromide                | g.  | 1.0  |
| Potassium iodide (0.1% solution) | cc. | 2    |
| Water to make one liter.         |     |      |

(pH was 10.1 at 70° F.)

The coatings were then washed for two minutes.

*Color development.*—The above coatings were given a reversal exposure for about 10 seconds (flash) with a No. 2 Photoflood set at a distance of 52 inches. The coatings were developed to an adequate D-max. in a developer having the following formula:

|                                  |     |      |
|----------------------------------|-----|------|
| Sulfuric acid (conc.)            | cc. | 1.5  |
| Sodium hexametaphosphate         | g.  | 0.5  |
| Sodium sulfite (anhydrous)       | g.  | 5.0  |
| Color developer <sup>1</sup>     | g.  | 0.6  |
| Sodium carbonate (monohydrate)   | g.  | 15.0 |
| Potassium bromide                | g.  | 0.25 |
| Potassium iodide (0.1% solution) | cc. | 2    |
| Coupler <sup>2</sup>             | g.  | 1.2  |
| Sodium hydroxide                 | g.  | 1.2  |
| Water to make one liter.         |     |      |

<sup>1</sup> 4-amino-3-methyl-N,N-diethylaniline hydrochloride.

<sup>2</sup> 2,4-dichloro-5-(p-toluenesulfonamido)-1-naphthol.

The coatings were washed for ten minutes and treated for two minutes in a silver bleach bath having the following composition:

|                          |     |    |
|--------------------------|-----|----|
| Potassium ferricyanide   | 100 | G. |
| Potassium bromide        | 10  |    |
| Borax                    | 7.5 |    |
| Boric acid               | 5.0 |    |
| Water to make one liter. |     |    |

The coatings were then treated for two minutes in a fixing bath having the composition given below, washed and dried.

|                                   |     |    |
|-----------------------------------|-----|----|
| Sodium thiosulfate (pentahydrate) | 200 | G. |
| Sodium sulfite (anhydrous)        | 10  |    |
| Water to make one liter.          |     |    |

In order to obtain cyan fog readings, an additional strip of each coating was put through the same process except that the flash reexposure was omitted. The D-max. and color (cyan) fog for each of the coatings were then measured, the results being given below.

Additional strips of coated emulsions were processed exactly as described above except that a formamidinothiomethyl compound, as identified above, and in the quantity given in the following table, was added to the color developer. The D-max. and cyan fog for each of these coatings were also measured, the results being given in the following table.

| Compound No. | Conc.,<br>g./liter | Coating Series A |             | Coating Series B |             |
|--------------|--------------------|------------------|-------------|------------------|-------------|
|              |                    | D-max.           | Cyan<br>Fog | D-max.           | Cyan<br>Fog |
| Control      | none               | 3.40             | 0.18        | 3.30             | 0.31        |
| (a)          | 0.15               | 3.10             | 0.03        | 3.30             | .06         |
| (b)          | 0.25               | no run           | no run      | 3.16             | .08         |
| (c)          | 0.30               | 3.50             | .07         | 2.90             | .11         |

The improvement obtained as a result of the use of one of the formamidinothiomethyl compounds of my invention is immediately apparent, in emulsions with or without a polyethyleneglycol derivative. While color

density is maintained at a high level, the color fog has been materially reduced.

While the advantages of my invention are particularly noticeable in cyan development, they are also quite noticeable in providing improved results in magenta and yellow development, as illustrated in the following examples.

#### Example 2

In a manner similar to that illustrated in Example 1 above, a portion of a gelatino-silver-bromide emulsion which had been sensitized with a sulfur compound and a gold compound of the type described above, and the oleyl ether of a polyethyleneglycol having a molecular weight greater than 300 (5 g./mole of AgX), was coated on a cellulose acetate support. The coating was exposed for  $\frac{1}{25}$  second to a 100-watt, 5400° K. light source on an Eastman Type 1b sensitometer. The exposed coating was then developed for 4 minutes in a developer having the following composition:

|                                  |     |      |
|----------------------------------|-----|------|
| Sodium tetraphosphate            | g.  | 0.5  |
| Potassium bromide                | g.  | 2.85 |
| Potassium iodide (0.1% solution) | cc. | 15   |
| Sodium bisulfite                 | g.  | 4.2  |
| N-methyl-p-aminophenolsulfate    | g.  | 4.5  |
| Sodium sulfite (anhydrous)       | g.  | 75.9 |
| Hydroquinone                     | g.  | 2.8  |
| Sodium carbonate (monohydrate)   | g.  | 27.5 |
| Hydroquinone sulfonate           | g.  | 1.9  |
| Isopropylamine                   | g.  | 6.43 |
| Water to make one liter.         |     |      |

The coating was then washed for two minutes.

*Color development.*—The above coating was given a reversal exposure for about 10 seconds (flash) with No. 2 Photofloods set at a distance of about 60 inches. The coating was developed 2 minutes in a color developer having the following composition:

|                                |      |    |
|--------------------------------|------|----|
| Sodium hexametaphosphate       | 0.5  | G. |
| Sodium sulfite                 | 5.0  |    |
| Color developer <sup>1</sup>   | 1.5  |    |
| Sodium carbonate (monohydrate) | 20.0 |    |
| Sodium bromide                 | 0.22 |    |
| Potassium iodide               | .002 |    |
| 6-nitrobenzimidazole nitrate   | .01  |    |
| Coupler No. 45                 | 0.5  |    |
| Sodium hydroxide               | 0.7  |    |
| Water to make one liter.       |      |    |

<sup>1</sup> 4-amino-3-methyl-N,N-diethylaniline hydrochloride.

The coating was washed for 10 minutes and treated for 2 minutes in a silver bleach bath having the composition given above. The coating was then rinsed and treated for 2 minutes in a fixing bath having the composition given above, washed and dried. A second strip was given the same treatment except that the flash reexposure was omitted. The D-max. and color (magenta) fog for the coating were then measured.

Another portion of the same emulsion was treated in exactly the manner described above, except that compound (a), as identified above, was added to the color developer (0.15 g./liter). The D-max. and magenta fog for this coating were also measured, the following tabulation showing the comparison between the untreated and treated coatings.

|                           | D-max. | Magenta<br>Fog |
|---------------------------|--------|----------------|
| Control                   | 1.85   | 0.67           |
| Compound (a) <sup>1</sup> | 1.87   | 0.16           |

<sup>1</sup> Development time—6 minutes.

#### Example 3

An ordinary gelatino-silver-bromide emulsion sensi-

tized with a sulfur sensitizer, a gold compound, and the oleyl ether of a polyethyleneglycol having a molecular weight greater than 300 (5.0 g./mole of AgX) was processed in exactly the manner described in Example 2 above, except that a yellow color-forming coupler was employed in place of the magenta developer of Example 2, while the concentration of compound (a) was reduced to 0.075 g./liter for the processing of the second coating. The time of color development for the first coating, the color developer containing no formamidinothiomethyl compound, was 8 minutes, while the development time for the processing of the second coating in the color developer containing compound (a) was 30 minutes. The yellow developer had the following composition:

|                              |       | G.   |
|------------------------------|-------|------|
| Sodium hexametaphosphate     | ----- | 0.5  |
| Sodium sulfite (anhydrous)   | ----- | 2.0  |
| Color developer <sup>1</sup> | ----- | 1.5  |
| Sodium bromide               | ----- | 0.22 |
| Potassium iodide             | ----- | .002 |
| 6-nitrobenzimidazole nitrate | ----- | .01  |
| Coupler No. 64               | ----- | 1.5  |
| Sodium hydroxide             | ----- | 0.4  |
| Water to make one liter.     | ----- |      |

<sup>1</sup> 4-amino-3-methyl-N,N-diethylaniline hydrochloride.

Measurement of the D-max. and yellow fog for each of the coatings gave the following results:

|              | D-max. | Yellow Fog |
|--------------|--------|------------|
| Control      | 1.23   | 0.36       |
| Compound (a) | 1.22   | 0.18       |

While it has been previously proposed to add various mercapto compounds to color developers, such compounds fail to maintain color density at a high level, although they do reduce color fog. For example, processing of an emulsion having the same composition as coating B of Example 1, the same developing compositions shown in Example 1 being used, except that 0.01 g./liter of 1-phenyl-5-mercaptopotetrazole was added to the color developer in place of the formamidinothiomethyl compound of Example 1, gave the following results:

|                                | Color Development, min. | D-max. | Cyan Fog |
|--------------------------------|-------------------------|--------|----------|
| Control                        | 4                       | 3.30   | 0.31     |
| 1-phenyl-5-mercaptopotetrazole | 5                       | 1.42   | 0.10     |

While the above mercapto compound did reduce the cyan fog to one-third the level of the coating treated with a color developer containing no antifogant, it also caused a density loss of more than one-half.

While the above examples primarily illustrate the use of photographic emulsions which have been chemically sensitized with the oleyl ether of polyethylene glycol, it is to be understood that other condensates of alkylene oxides can be advantageously employed to sensitize such emulsions. Such condensates are generally referred to as alkylene oxide polymers, the alkylene oxides generally containing from 2 to 4 carbon atoms. Such alkylene oxide polymers include polyalkylene glycols and condensation products of alkylene oxides with organic compounds containing an active hydrogen atom, such as alcohols, amines, mercaptans, acids, amides, etc. Generally, such alkylene oxide polymers have a molecular weight of at least 300, as shown in U. S. application Serial No. 550,495, mentioned above. It is to be further understood that the emulsions employed in my invention need not be chemically sensitized, although particularly useful results have been obtained with emul-

sions which have been chemically sensitized with such alkylene oxide polymers.

The formamidinothiomethyl compounds useful in my invention can be added to the color developers either in the form of their free bases or in the form of acid-addition salts of these bases. Since the color developing solutions of my invention are strongly alkaline, the acid-addition salts are converted to the free bases, in which form they manifest their activity. It is to be understood that the term "formamidinothiomethyl" compound includes not only the free bases but also acid-addition salts of these bases.

As mentioned above, the compounds of Formula I can be prepared according to methods previously described in the prior art. For example, compound d above was prepared as follows:

*Example A.—S-carbethoxymethyl - 1 - phenyl - 3 - (4H-1,2,4-triazol-3-yl)isothiourea*

3-amino-1,2,4-triazole was boiled in dry dioxane with an equimolecular amount of phenyl isothiocyanate. There was obtained a 50 to 60 percent yield of the desired 1-phenyl-3-(3-triazolyl)thiourea as a white solid which was only slightly soluble in water and dioxane, but was readily soluble in dimethylformamide. It was recrystallized from its solution in dimethylformamide by addition of water to give white crystals melting at 230-234° C.

The above thiourea compound was refluxed for 2 to 4 hours with ethyl chloroacetate in dry dioxane, yielding pale yellow solid which melted gradually with decomposition above 280° C. Recrystallization of this solid from dimethylformamide yielded S - carbethoxymethyl - 1-phenyl - 3 - (4H - 1,2,4 - triazol - 3 - yl) - isothiourea as a solid melting at 296-302° C. with decomposition.

Compound c above was prepared according to the directions given in "Jour. Am. Chem. Soc.," vol. 77 (1955), page 6231.

As mentioned above, the color-forming compounds of my invention can be prepared according to methods previously described in the literature. The following two examples will serve to illustrate methods of preparing two typical couplers useful in my invention.

*Example B.—N-benzoylaceto-o-anisidine*

A two-liter flask was fitted with a one-holed rubber stopper and a steam-jacketed Friedrichs condenser. To the top of this condenser was fitted a standard distillation head, thermometer and downward pointing Liebig condenser cooled with water. The flask was then charged with 600 cc. of neutral histological xylene, 74 g. (0.6 mol.) of o-anisidine and 115 g. (0.6 mol.) of ethyl benzoylacetate. The flask was refluxed for 90 minutes at such a rate that most of the boiling xylene condensed in the steam-jacketed condenser, but some distillate was condensed in the cold condenser. The temperature at the top of the hot condenser was 110° C. at the beginning of the reflux period, but slowly dropped to 70° C. at the end of the period. During this time, 45 cc. of distillate was collected from the cold condenser. The heating mantle was turned off, 500 cc. of ligroin was added to the hot solution, and the material allowed to cool for 16 hours. The resulting crystalline product was broken up, filtered off and air-dried. A yield of 90 g. of crude product was obtained, M.P. 86-8° C. Recrystallization of the product from 520 cc. of methanol yielded 76.3 g. of product, M.P. 86-8° C. Yield was 47.4 percent of theory.

*Example C.—3-(p-nitrophenoxyacetylarnino)-1-(2',4',6'-trichlorophenyl)-5-pyrazolone*

A two-liter round-bottomed flask equipped with a condenser and a mechanical stirrer, was charged with 450 cc. of acetonitrile, 32 g. (0.1 mol.) of 1-(2,4,6-trichlorophenyl)-3-amino-5-pyrazolone (U.S. Patent 2,600,788),

and 27 g. (0.13 mol.) of p-nitrophenoxyacetyl chloride. The mixture was refluxed on the steam bath for three and one-half hours with good stirring, complete solution occurring when reflux temperature was attained. At the end of the reflux period, the crystalline product, which had separated from the refluxing mixture, was suction-filtered from the hot mother liquors. It was then washed on the funnel with successive portions of acetonitrile, ethanol, water, ethanol, and ether. After drying overnight in a steam cabinet, there were obtained 47 g. (89% of theory) of the desired product as a white solid, M.P. 244-6° C.

The p-nitrophenoxyacetyl chloride used above was prepared as follows: In a 500-ml. flask were mixed 19.7 g. (0.1 mole) of p-nitrophenoxyacetic acid and 100 ml. of thionyl chloride. The mixture was refluxed for 5 hours on a steam bath and the excess thionyl chloride removed under reduced pressure. The removal of the thionyl chloride was continued until the residue had reached constant weight. The acid chloride was used without purification and gave good results. It can be crystallized from dried ligroin to obtain a white crystalline material melting at 86-87° C.

The p-nitrophenoxyacetic acid used above was prepared as follows: In a 5-liter flask were placed 278 g. (2 moles) of p-nitrophenol, 190 g. (2 moles) of chloroacetic acid, 168 g. (4.2 moles) of sodium hydroxide and 2 liters of water. The mixture was boiled in the open flask until it showed a neutral reaction to litmus paper. The reaction temperature reached 115° C. and some water was evaporated. When the neutral point had been reached (2.5-3 hours) an additional 84 g. (2.05 moles) of sodium hydroxide and 95 g. (1 mole) of chloroacetic acid were added to the flask and the heating continued until a neutral reaction again resulted.

To the cooled reaction mixture were added 500 ml. of concentrated hydrochloric acid with stirring. The solid formed was filtered, slurried with 3 liters of ice cold water and again filtered and washed with 1 liter of ice cold water. The dry product melted at 182-184° C. and weighed 300 g. Yield was 76% of the 394 g. theory. It can be crystallized from denatured alcohol, if desired.

What I claim as my invention and desire secured by Letters Patent of the United States is:

1. A developing composition for color photography comprising an arylenediamine color developer and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub> represents a member selected from the group consisting of a carbalkoxyl group containing from 2 to 5 carbon atoms, an alkyl group containing from 1 to 4 carbon atoms, a tetrazaindenyl group, a pyridyl group, and an aminocarbonyl group.

2. A developing composition for color photography comprising alkali, an alkaline sulfite, a p-phenylenediamine color developer, and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub>

represents a member selected from the group consisting of a carbalkoxyl group containing from 2 to 5 carbon atoms, an alkyl group containing from 1 to 4 carbon atoms, a tetrazaindenyl group, a pyridyl group, and an aminocarbonyl group.

3. A photographic developer for color photography comprising a strongly alkaline solution of a p-phenylenediamine photographic developing agent, an alkali metal sulfite and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub> represents a member selected from the group consisting of a carbalkoxyl group containing from 2 to 5 carbon atoms, an alkyl group containing from 1 to 4 carbon atoms, a tetrazaindenyl group, a pyridyl group, and an aminocarbonyl group.

4. A developing composition for color photography comprising a p-phenylenediamine color developer, an alkali metal sulfite, and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub> represents a member selected from the group consisting of a carbalkoxyl group containing from 2 to 5 carbon atoms, an alkyl group containing from 1 to 4 carbon atoms, a tetrazaindenyl group, a pyridyl group, and an aminocarbonyl group.

5. A developing composition for color photography comprising a p-phenylenediamine color developer, an alkali metal sulfite, and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub> represents a tetrazaindenyl group.

6. A photographic developing composition for color photography comprising a p-phenylenediamine color developer, an alkali metal sulfite, and 2-formamidinothiomethyl-4-hydroxy-6-methyl-1,3,3a,7-tetrazaindenyl.

7. A developing composition for color photography comprising a p-phenylenediamine color developer, an alkali metal sulfite, and bis(2-formamidinothiomethyl-6-methyl-1,3,3a,7-tetrazaindenyl-4-yl)sulfide.

8. A developing composition for color photography comprising a p-phenylenediamine color developer, an alkali metal sulfite, and 2-S-thiouroniummethanesulfonate.

9. A developing composition for color photography comprising a p-phenylenediamine color developer, an alkali metal sulfite, and S-carbethoxymethyl-1-phenyl-3-(4H-1,2,4-triazol-3-yl)isothiourea.

10. A developing composition for color photography comprising a p-phenylenediamine color developing compound, an alkali metal sulfite, a color-forming compound capable of coupling with the oxidation products of said p-phenylenediamine color developing compound to produce a colored image selected from the group consisting

**13**

of cyan, magenta and yellow, and a compound selected from those represented by the following general formula:



wherein R represents a member selected from the group consisting of a hydrogen atom, an alkyl group containing from 1 to 3 carbon atoms, and a monocyclic aryl group of the benzene series containing from 6 to 7 carbon atoms, R<sub>1</sub> represents an amino group, and R<sub>2</sub> represents a member selected from the group consisting of a car-

5

balkoxyl group containing from 2 to 5 carbon atoms, an alkyl group containing from 1 to 4 carbon atoms, a tetrazaindenyl group, a pyridyl group, and an aminocarbonyl group.

10

**14**

References Cited in the file of this patent

## UNITED STATES PATENTS

- |           |                     |               |
|-----------|---------------------|---------------|
| 2,252,718 | Mannes et al. ----- | Aug. 19, 1941 |
| 2,453,087 | Dersch et al. ----- | Nov. 2, 1948  |
| 2,514,650 | Knott et al. -----  | July 11, 1950 |